

May 10, 1927.

1,627,682

J. F. WYZALEK

# METHOD AND APPARATUS FOR HEAT TREATING STEEL ARTICLES

Filed March 14, 1924



Fig. 1.



Fig. 4.



Fig. 7.



Fig. 5. Fig. 6.



٣٦



Fig. 2.



३५६

INVENTOR.  
JOHN F. WYZALEK.

BY  
F. L. D. D. M. D.  
his ATTORNEY.

Patented May 10, 1927.

1,627,682

# UNITED STATES PATENT OFFICE.

JOHN F. WYZALEK, OF ARLINGTON, NEW JERSEY, ASSIGNOR TO GENERAL MOTORS CORPORATION, OF DETROIT, MICHIGAN, A CORPORATION OF DELAWARE.

## METHOD AND APPARATUS FOR HEAT TREATING STEEL ARTICLES.

Application filed March 14, 1924. Serial No. 699,835.

This invention relates to the heat treatment of steel articles and is herein illustrated by reference to a method and apparatus for heat treating race rings for roller bearings.

A race ring for a ball or roller bearing must be composed of steel having different properties at different portions of the article. The roller engaging portion must be very hard to resist wear and abrasion but the ring as a whole, having to stand shock and overloads in service and grinding strains in manufacture, must be tough without being brittle. The roller engaging portions of race rings are therefore case hardened while other portions are of low carbon content. As is well known, to refine the grain of a low carbon steel, it must be heated to a higher temperature than a high carbon steel. If a race ring is heated above the critical range for the low carbon steel and quenched, the low carbon portion or "core" becomes well refined but the case hardened portion or "case" acquires a coarse grain. This must be removed by another heat treatment at a temperature above the critical range for the high carbon but not high enough to materially affect the already refined grain of the core.

An object of this invention is to provide improved hardening apparatus which will avoid the expense incident to the separate handling of the articles for the second heat treatment. Another object is to provide improved apparatus of this character which will economize heat by eliminating the first quenching in liquid and the subsequent reheating of the articles from quenching temperature. Another object is to simplify the heat treatment and increase production by heat treating articles of varying carbon content as a continuous uninterrupted operation. In accomplishing these and other objects, the articles are fed in a stream, first through one furnace to heat them above the critical range for the low carbon "core," then cooled below the critical range for the low carbon core, then, without further cooling or quenching in liquid, are continuously passed through a second furnace to heat the

articles above the critical range for the high carbon portion, and finally quenched in liquid.

To these ends and also to improve generally upon devices of the character indicated my invention consists in the various matters hereinafter described and claimed.

Referring to the drawings, Figure 1 is a side elevation of the apparatus partly in section.

Figure 2 is a section on the line 2—2 of Figure 1.

Figure 3 is an enlarged view of the connecting tube section between the furnaces.

Figure 4 is a section on the line 4—4 of Figure 3.

Figure 5 is a section on the line 5—5 of Figure 6.

Figure 6 is a vertical section of a jacketed connecting tube.

Figure 7 is an end view of Figure 6 and

Figure 8 is a side elevation of a modification.

The numeral 10 indicates a frame or support for furnaces 12 and 14 which are spaced from one another in end to end relation.

The furnaces may be identical and are composed of the usual refractory material and have ports 16 through which oil fuel may be admitted. Extending longitudinally through the heating chamber of each furnace are guides 18, herein shown as tubes through

which steel articles are fed in a stream, the tubes protecting the articles from contact with the products of combustion. The tubes are carried on supports 20 of refractory material and have flattened faces 22 meeting at the bottom to support and guide the articles.

When the articles are steel race rings, they engage the flat faces at two points and are less likely to move laterally while being fed. Each guide or tube 18 has flanges 24 at the ends, the adjacent flanges on the tubes of the two furnaces being bolted to similar flanges 26 at the ends of a connecting tube section 28.

Suitable gaskets 30 of heat insulating material are interposed between the connecting flanges and the connecting section 28 is provided with a series of peripheral cooling fins 32 to facilitate extraction

100

95

90

85

80

75

70

65

60

of heat by the atmosphere from the articles being fed through the tubes. The tube sections 28 also have flattened faces 34 meeting at the bottom and these align with the flattened faces 22 on the furnace tubes to furnish an uninterrupted guideway through the apparatus.

A reciprocating plunger 36 pushes the articles in a stream from a guide 38 into the furnace tubes and feeds them continuously and uninterruptedly through the furnaces to a tank 40 of liquid where they are quenched. The first furnace 12 is heated to a temperature above the critical range for the low carbon portions of the articles, then the articles are cooled in the connecting section below the critical range and, without any quenching in liquid, are then carried through the second furnace which heats them above the critical range for the high carbon portions of the articles but not high enough to materially affect the low carbon portions. Then they are quenched in liquid in the tank 40.

25 In the form of the invention shown in Figures 5 to 7, there are two connecting tubes 42 surrounded by a casing 44 to form a jacket, any suitable fluid such as air or water being admitted at the inlet 46 and discharged at the exit opening 48. The end walls of the jacketed section have tapped openings 50 to receive screws passing through the flanges on the ends of the furnace tubes.

35 In Figure 8 there is shown means for varying the cooling effect of the connecting tube fins. Numeral 52 indicates a lower section which is bolted at its ends as before to the ends of the furnace tubes. An upper section 54 normally rests on the lower section but can be raised vertically to allow access of the atmosphere through the slots thus formed. Lugs 56 on the lower section receive the threaded portions 58 of hand screws which pass also through lugs 62 on the upper section, there being collars 60 on the screws 58 to support the upper section in different positions of adjustment for varying the size of the slots.

45 Although the invention has been illustrated by reference to specific steps and apparatus, it should be understood that, in its broader aspects, the invention is not necessarily limited to the details set forth.

55 I claim:

1. Apparatus for heat treating steel articles, having, in combination, a furnace having a tube extending through the heating chamber, a second furnace spaced from the first and having a tube extending through the heating chamber, and an unheated tube section joining said furnace tubes; substantially as described.

2. Apparatus for heat treating steel articles, having, in combination, a furnace hav-

ing a tube extending through the heating chamber, a second furnace spaced from the first and having a tube extending through the heating chamber, a tube section joining said furnace tubes, said tube section having peripheral cooling fins to increase the radiating surface; substantially as described.

3. Apparatus for heat treating steel articles, having, in combination, a furnace having a tube extending through the heating chamber, a second furnace spaced from the first and having a tube extending through the heating chamber, an unheated tube section connecting said furnace tubes, and heat insulating material at the joint between said unheated tube and the furnace tubes; substantially as described.

4. Apparatus for heat treating steel articles, having, in combination, a furnace having tubes extending through the heating chamber, a second furnace spaced from the first and having tubes extending through the heating chamber, and a plurality of tube sections joining said furnace tubes, said tube sections being transversely connected by flanges forming cooling fins; substantially as described.

5. Apparatus for heat treating round articles, having, in combination, a furnace having a guide extending through the heating chamber, a second furnace spaced from the first and having a guide extending through the heating chamber, a tube section joining said furnace guides, said tube section having flattened portions meeting at the bottom to support the articles at two points and guide the same; substantially as described.

6. Apparatus for heat treating round articles, having, in combination, a furnace having a tube extending through the heating chamber, said tube having flattened portions meeting at the bottom to support the articles at two points, and means for pushing the articles through the tube in a stream; substantially as described.

7. Apparatus for heat treating steel articles, having, in combination, a furnace having a guide extending through the heating chamber, a second furnace spaced from the first and having a guide extending through the heating chamber, and an unheated tube section joining said guides, said tube section having means to vary the cooling effect; substantially as described.

8. Apparatus for heat treating steel articles of high carbon content at one portion and lower carbon content at other portions, having, in combination, a heating chamber for heating the articles above the critical range for the low carbon portion, a chamber for cooling said articles slightly below the critical range, a second heating chamber for receiving and heating said articles

above the critical range for the high carbon portion, and means for quenching said articles; substantially as described.

9. Apparatus for heat treating steel articles of high carbon content at one portion and lower carbon content at other portions, having, in combination, a heating chamber, a second heating chamber spaced from the

first and heated to a lower temperature, a covered cooling chamber connecting said heating chambers, and means for feeding articles through said chambers in a continuous stream; substantially as described.

In testimony whereof I hereunto affix my signature.

JOHN F. WYZALEK.